

# UNITED STATES PATENT OFFICE.

CHARLES IGNATIUS GOESSMANN, OF WORCESTER, MASSACHUSETTS,  
ASSIGNOR TO VELLUMOID PAPER COMPANY, OF AMHERST, MAS-  
SACHUSETTS, A CORPORATION OF WEST VIRGINIA.

## PAPER CHARACTERIZED BY ITS IMPERVIOUS NATURE AND STRENGTH.

No. 804,808.

Specification of Letters Patent.

Patented Nov. 14, 1905.

Original application filed August 16, 1900, Serial No. 27,086. Divided and this application filed February 24, 1903. Serial No. 144,807.

*To all whom it may concern:*

Be it known that I, CHARLES IGNATIUS GOESSMANN, a citizen of the United States of America, and a resident of Worcester, in the county 5 of Worcester and Commonwealth of Massachusetts, have invented new and useful Improvements in Paper Characterized by Its Imper-  
10 pious Nature and Strength, (this application being a division of an application filed by  
me in the United States Patent Office August 16, 1900, Serial No. 27,086,) of which the following is a specification.

My invention relates particularly to paper the product resulting from novel treatment 15 either during the primary process of manufacture into paper or after the same has been manufactured, such treated paper possessing a texture which has been greatly strengthened and being as a whole rendered substan-  
20 tially impervious to water, moisture, grease, acid, &c.

The objects of my invention are, first, to produce a paper which is stronger than other products of a similar nature; second, to provide a paper which is non-absorbent of water 25 or moisture, or, in other words, substantially waterproof; third, to provide a paper which is non-absorbent of grease, or, in other words, grease-proof; fourth, to provide a paper which 30 is non-absorbent of acids, or, in other words, acid-proof; fifth, to furnish a paper which is a non-conductor of electricity; sixth, to furnish a paper suitable for packing joints in pipes and connections; seventh, to produce a 35 hygienic paper, and, eighth, to produce paper possessing any or all of these advantages in a greater and more marked degree than has been heretofore done.

My invention consists of the product after 40 the paper has been treated in accordance with the method or process hereinafter described, and I attain the objects of my invention, both singly and collectively, as hereinafter set forth.

45 In carrying out my invention any convenient and appropriate machinery or apparatus may be employed; but the best and only known method for producing this paper is described as follows: The treatment may be applied 50 while the pulp is being formed into paper, or the finished paper may be treated. If the material is to be treated while being formed into paper, then the better method is to be-

gin the treatment when the web of pulpy material leaves the Fourdrinier wire or the cyl- 55 inders, it then being in a damp condition, but with the larger percentage of moisture removed. From this point the treatment of the paper is the same whether it be pulp in a sheet, as above stated, or finished paper. 60

The treatment consists, first, in saturating the paper with glutinous material, preferably animal glue, and by preference the bath of glutinous material should be hot to effect the more rapid absorption and more perfect per- 65 meation, impregnation, and deposit of the glu-  
tinous material within all the microscopic interstices throughout the body of the paper being treated. By preference a suitable tank 70 is provided in which the glutinous material is deposited and in which it may be kept heated to a constant temperature, the paper being passed through the tank and saturated during its passage. I prefer that the material being treated be kept in motion and pass in a con- 75 tinuous sheet—that is, be fed from a roll and the finished product be wound in a roll after final treatment—this saves time, and I find that the requisite permeation or incorporation of glutinous matter in the fiber will with some 80 papers—for instance, lightly-sized Manila hemp—require but a few seconds. As the paper passes from the glutin-tank the surplus of glutinous matter is removed from the sur- 85 face by mechanical means as contradistin- guished from simply allowing it to pass off by gravity, and in most instances I prefer to pass the paper between suitable pressure-rolls to remove such surplus. The strength and 90 consistency of the glutinous bath may be va-  
ried, depending upon the material being treated and the uses for which such material is de- 95 signed. It may, however, be stated that in a majority of cases a hot solution of about one part of animal glue to about ten parts of water, by weight, gives the best results. After leaving the bath of glutinous material and having the surplus adhering to the sur- 100 faces removed the paper before drying is passed into or through a solution of formaldehyde and water to "set" the glutinous ma-  
terial. The strength of this solution may also be variable, depending, as heretofore stated, upon the paper and uses for which it is designed. In the majority of cases, how- 105 ever, a solution of one part of formaldehyde

(thirty-five-per-cent. solution) to five parts of water, by weight, gives the best results, and the best result is attained if this bath is cold instead of hot, though any particular temperature is not essentially necessary. The effect of the formaldehyde solution upon the glutin-saturated paper is to precipitate the glutinous matter and render it insoluble.

As the material comes from the formaldehyde-bath I prefer that the surplus adhering to the surfaces be removed by mechanical means, pressure-rolls being probably most convenient. The paper is then dried in any convenient manner. The best result in drying, so far as I am at present advised, is attained by the air-blast—*i. e.*, projecting blasts of air against both surfaces of the paper. This drying removes all the watery constituents and leaves the paper in a toughened or greatly strengthened condition, but not in practical condition for commercial uses, as it is brittle, horny, and stiff and has an objectionable odor and taste on account of the presence of the aldehydes, paraldehydes, formic acid, and other products, the result of oxidation, hence needs to be "tempered." Now while the glutinous material is rendered insoluble—that is, it is so acted upon by the formaldehyde and the chemical action which takes place while the united solutions are giving off their watery constituents that it will not fully dissolve—it is, however, in a condition to be acted on by moisture, as it will swell and absorb or take up permanently by either chemical or mechanical action a percentage of water and will also become improved in many respects, so that to temper and render the paper soft and pliable and adapt it for most commercial uses I subject it to moisture, which penetrates the paper, causing a swelling in all directions, filling the interstices perfectly and resulting in "hydration" throughout the entire cellular structure. Two actions, mechanical and chemical, appear to take place, the mechanical action being the temporary absorption of water analogous to the absorption of water by a dry sponge, the chemical action being the permanent union of water with the treated paper, analogous to the union of water and tapioca, causing swelling, or like the chemical combination of water with lime or cement. For this purpose I prefer to pass the paper into a bath of hot water, saturated steam, or equivalent heat-and-moisture medium, thus causing the fibers and the non-soluble glutinous material filling the interstices to expand in all directions and forcing the glutinous material into all the microscopic pores or openings and into the masses of fiber, causing a commingling or thorough incorporation of the fibers and the glutinous compound, and at the same time, as heretofore indicated, a change (hydration) takes place, whereby the hardened mass of fiber, glutinous material, and formaldehyde becomes

tempered and softened and the strength imparted by the previous treatment increased. To heighten the tempering and softening effect, I may in some instances introduce glycerin in the tempering-bath, and in most cases one two-hundredths in volume of glycerin gives the best results.

The paper may be dried in any convenient manner and is in condition for most commercial uses, it being greatly strengthened, more flexible, more impervious to moisture, acids, grease, or alkalies, and is suitable for the manufacture of binding-twine, carpets, and many novelties, for dry wrappings and lining packing-cases, &c., but is liable to have a disagreeable taste and may carry traces of acids, rendering it impracticable for some uses—for instance, wrapping butter, meats, cheese, &c.—after receiving the alkali treatment. The paper is also valuable as a packing for joints in steam, water, and other pipes or connections. For the purpose, therefore, of rendering the material absolutely free from all traces of acidity and all taste and odors and, in fact, to render it absolutely hygienic I pass it through a bath of water and a volatile alkali, (ammonium hydrate,) the proportion by preference in a majority of cases being one one-hundredth of ammonium hydrate to ninety-nine one-hundredths of water by volume, and I may add a small percentage of wood-alcohol. This bath is preferably cool; but a variation in its temperature will not to a serious extent interfere with the results. The effect of this bath followed by drying is to complete the chemical reaction and destroy all taste or odor, removing all traces of acids and rendering the paper hygienic in all respects. The material may be calendered or cut and used for any of the purposes desired. If the material is to be subjected to the volatile-alkali bath, it is not necessary to dry it between the tempering and volatile-alkali baths.

The paper made in accordance with the foregoing will be found to be greatly strengthened, some materials being increased in strength from one hundred to seven hundred per cent. It will be non-absorbent to acids, greases, and alkalies and substantially waterproof, and owing to its component integrate structure will be practically non-conductive to electricity, adapting it as a superior insulating material, and may with perfect safety be employed for wrapping butter, meats, spices, groceries, and all materials whether unctious or otherwise.

By the term "hydration" as used herein I mean the subjecting of the material (after treatment with glutinous material and formaldehyde and drying) to moisture, whereby the action herein described takes place.

A sheet or web of paper can be treated by the hereinbefore-described process as rapidly as it is manufactured, as the time for exposure to the action of the glutinous material need

not be longer than the time required for it to become saturated, this of course varying with different thicknesses and densities, and the length of time of exposure may be fixed 5 without checking the speed by making the tank of such length that the requisite time will elapse while the sheet is passing through it and the guides so arranged as to maintain the sheet in position to be acted on by such 10 solution the requisite length of time. I find four seconds exposure to the action of formaldehyde sufficient in most cases.

Having, therefore, described my invention, what I claim, and desire to secure by Letters 15 Patent, is—

1. A paper with its cellular structure permeated and impregnated with a formaldehyde-

treated glutinous material permanently and insolubly incorporated therewith, the whole being softened by hydration. 20

2. A sheet of fibrous material with its interstices filled with a glutinous substance that has been "set" before being dried and thereafter dried and "tempered" by hydration, the whole constituting a corporeal mass of 25 united tissue throughout.

In testimony whereof I have signed my name to this specification in the presence of two subscribing witnesses.

CHARLES IGNATIUS GOESSMANN.

Witnesses:

F. A. CUTTER,  
GUSTAVE GOEDIKE.